

## UNITED STATES PATENT OFFICE

2,237,829

## METHOD OF DYEING

Winfield Walter Heckert, Ardentown, Del., assignor to E. I. du Pont de Nemours & Company, Wilmington, Del., a corporation of Delaware

No Drawing. Application February 5, 1938,  
Serial No. 188,931

1 Claim. (Cl. 8—24)

This invention relates to the coloring of mixed textile materials consisting of textile material comprising an organic derivative of cellulose textile material and textile material of different chemical constitution, and it especially relates to the coloring of mixed textile fabrics wherein the textile material comprising an organic derivative of cellulose has previously been modified in dyeing characteristics by means of a polymeric compound containing in its structure amino nitrogen. Such polymeric compounds are described in Heckert application, Serial No. 143,829 Patent No. 2,191,887, of which the present application is a continuation-in-part.

Yarns and fabrics of organic derivatives of cellulose, especially of cellulose esters, such as cellulose acetate, are generally non-receptive to acid dyestuffs which are commonly used to dye woolen fabrics. The same is also true of direct dyestuffs which are commonly used to dye cotton or regenerated cellulose fabrics as well as a great many other dyestuffs commonly employed to dye woolen, silk, cotton or regenerated cellulose goods. Vice versa, the dyestuffs specially developed for use on cellulose acetate materials have relatively little dyeing affinity for woolen, silk, cotton or regenerated cellulose goods. Commercially, advantage of this selectivity in dyeing properties has been taken to produce cross dyeing effects since one or the other of the mixed fibers is left undyed and may later be colored with an appropriate dyestuff. The selectivity in dyeing properties, however, is a disadvantage when it is desired to color all component fibers in a mixed fabric containing cellulose acetate, and becomes markedly so when it is desired to dye the mixed fabric to a uniform solid color. In such cases, it is necessary to employ relatively time-consuming and expensive procedures, for instance in one of the present commercial procedures for dyeing a cellulose acetate containing mixed fabric a solid uniform color, the mixed fabric is dyed with a bath containing a dyestuff for the cellulose acetate, and then is withdrawn and dyed in a bath containing a dyestuff for the other yarn component in the fabric, each dye being carefully selected so as to dye one type of fiber and not the other.

One object of the instant invention is, therefore, to simplify and render less expensive the dyeing of mixed textile fabrics consisting of organic cellulose derivative yarns and wool, silk, cotton, or regenerated cellulose yarns.

Another object of the invention is to produce a uniformly solid colored mixed textile fabric con-

taining wool, silk, cotton, or regenerated cellulose yarns and organic cellulose derivative yarns with a dye having an affinity for wool, silk, cotton, or regenerated cellulose yarn, but substantially no affinity for unmodified organic cellulose derivative yarn.

A further object of the invention is to uniformly and solidly color throughout mixed textile fabrics containing cellulose acetate yarns by means of a dye bath containing only a dye or dyes having no affinity for unmodified cellulose acetate.

The above and other objectives are accomplished by the process of the present invention consisting of modifying cellulose acetate yarns with a polymeric compound containing amino nitrogen, forming the modified cellulose acetate thread into a mixed textile fabric with wool, silk, cotton, or regenerated cellulose yarns by means of standard textile operations, and coloring the mixed textile fabric throughout by treating the same under controlled conditions in a dye bath containing only a dye or dyes having an affinity for the wool, silk, cotton, or regenerated cellulose fibers but substantially none for unmodified cellulose acetate.

In accordance with the preferred manner of carrying out the invention, the following steps may be taken. Cellulose acetate yarns are spun under such conditions that the spun yarns contain by weight 3 to 15% of a polymeric compound containing amino nitrogen, such as a polymerized amino alcohol ester of an acrylic acid such as alpha-methacrylic. The modified cellulose acetate yarns are woven with wool, silk, cotton, or regenerated cellulose yarns into a mixed textile fabric and the mixed fabric is entered in a dye bath containing a dyestuff or dyestuffs having no affinity for unmodified cellulose acetate, but possessing affinity for the other fiber in the mixed fabric. The concentration, temperature, and pH of the dye bath and time of immersion of the fabric therein are so regulated that the entire mixed fabric, including the modified cellulose acetate yarn, is dyed to a uniform level solid color.

A few examples will now be cited in order to facilitate comprehension of the operation of the invention. It will be understood the examples are illustrative only, and are not to be considered limitative.

EXAMPLE I.—(One bath, one temperature, neutralized midway)

Polymerized beta-diethylaminoethyl alpha-methacrylate, prepared as described in Example

B of Heckert application Serial No. 143,829 is dissolved in acetone and to this solution sufficient cellulose acetate is added to form a spinning solution containing 20% cellulose acetate, 2% polymer, and 78% acetone. The solution is dry spun into fibers which are fabricated by standard methods into a crepe fabric, the warp of which consists of modified cellulose acetate fibers and the filling of regenerated cellulose threads. The resulting fabric is submitted to an aqueous scouring bath and entered cold into a dye bath having a 40:1 ratio of liquor volume to fabric weight and containing 2% of a green direct cotton dyestuff of Color Index No. 594, 20% Glauber's salt, and 2.5% acetic acid. With frequent turning of the fabric, the temperature of the dye bath is raised quickly to about 85° C. and held there for twenty minutes after which soda ash is added to neutralize the acidity of the dye bath. After neutralization, the fabric is dyed in the bath at about 85° C. for another 20 minutes with frequent turning, and then is withdrawn, rinsed, and dried. Viewed in piece, the mixed fabric is found to be dyed throughout a uniform level solid green.

Instead of neutralizing the dye bath, one may somewhat less desirably use two dye baths, the first containing 20% Glauber's salt, 2.5% acetic acid, and 1.2% of the green direct cotton dyestuff and the second being neutral and containing 20% Glauber's salt and .8% of the green direct cotton dyestuff. In such case, the mixed fabric is kept in the first bath at about 85° C. until substantially all the dyestuff is exhausted, after the mixed fabric is withdrawn, rinsed, and entered in the second bath which is quickly raised to a temperature of about 85° C. The fabric is frequently turned and after dyeing for about 20 minutes at a temperature of about 85° C. is withdrawn from the substantially exhausted dye bath, rinsed, and dried.

**EXAMPLE II.—(Buffered, one dye and bath)**

A crepe fabric, consisting of a warp of cellulose acetate yarns containing 10% polymerized beta-diethylaminoethyl alpha-methacrylate, and a filling of regenerated cellulose yarns, after an aqueous scouring treatment, is entered cold in a dye bath containing 2% of a red direct cotton dyestuff of Color Index No. 278, 15% Glauber's salt, 20% monosodium phosphate, and 26% of disodium phosphate. The ratio of liquor to weight of fabric is 40:1. The temperature of the dye bath is raised to a temperature of 85-90° C. during the space of 15 minutes and the dyeing is continued at that temperature for 45 minutes with frequent turning of the crepe fabric piece. The crepe regenerated cellulose-modified cellulose acetate fabric piece is then removed from the dye bath, rinsed and dried. The fabric piece is dyed a uniform level solid red.

**EXAMPLE III.—( $(NH_4)_2C_2H_3O_2$ , viscose rayon-acetate-diazo)**

Cellulose acetate yarns containing 10% of polymerized beta-diethylaminoethyl alpha-methacrylate, are incorporated as warp of a crepe fabric in which the filling consists of regenerated cellulose threads. After treatment with the usual aqueous scouring bath, the mixed fabric is entered at about 50° C. in a dye bath having a 40:1 ratio of liquor volume to fabric weight and containing 2% of a blue developable dye of Color Index No. 317, 5% of sodium chloride, and 8% of neutral ammonium acetate. The temperature of the dye bath is next quickly raised to about 85°

70 C. and maintained at that temperature for 30 to 40 minutes while frequently turning the fabric. The mixed fabric is then removed from the dye bath, rinsed well, and entered into a diazotizing bath at a temperature of 18-24° C. and containing 3% sodium nitrite and 4% sulfuric acid. After a diazotizing treatment of 20 minutes with occasional turning, the mixed fabric is quickly but thoroughly washed with water and introduced into a developing bath containing 1% beta naphthol as a developer and .5% sodium hydroxide. After treatment with the developing bath for a period of 20 minutes, the mixed fabric is rinsed thoroughly, squeezed out, and dried. The mixed fabric piece is dyed throughout a uniform level solid blue.

**EXAMPLE IV.—(Cotton-one dye)**

Cellulose acetate staple fibres, containing 5% of polymerized beta-diethylaminoethyl alpha-methacrylate, are mixed with cotton, and after being duly processed into a sliver and thread, are woven into a fabric consisting approximately of 50% modified cellulose acetate and 50% cotton. 20 After the customary aqueous scouring boil-off, the mixed fabric is entered at 50-60° C. in a dye bath containing 1% of a red direct cotton dyestuff of Color Index No. 278,  $\frac{1}{4}$ % acetic acid, and 15% Glauber's salt. The temperature of the dye 25 bath is raised during the course of 15 minutes to 85° C. and the dyeing is continued at this temperature for 45 minutes with frequent turning of the mixed fabric. The cotton-cellulose acetate fabric piece is then removed, and after rinsing and drying 30 is found to be dyed a uniform level solid red.

**EXAMPLE V.—(Cotton-developed dye)**

Cellulose acetate staple fibres, containing 10% of polymerized beta-diethylaminoethyl alpha-methacrylate, are mixed with cotton and thereafter are processed by standard textile procedure into a fabric consisting of 50% modified cellulose acetate and 50% cotton. The mixed fabric piece is dyed a uniform level solid blue by dyeing with 40 a blue developable dyestuff of Color Index No. 317 following the same procedure outlined in Example III.

**EXAMPLE VI.—(Wool-acid dye)**

Cellulose acetate staple fibres, containing 5% of polymerized beta-diethylaminoethyl alpha-methacrylate, are mixed with wool fibres and the mixture converted by standard textile operations into a fabric consisting of 50% wool and 50% modified cellulose acetate. After an aqueous scouring treatment, the wool-cellulose acetate fabric is entered cold in a dye bath containing 1% of a red wool acid dye of Color Index No. 430, 15% Glauber's salt, 5% monosodium phosphate, 45 and 13% disodium phosphate. The dye bath has a pH of about 6.7 and a ratio of liquor volume to weight of fabric of 40:1. The temperature of the dye bath is brought to 85-90° C. within 15 minutes, and the dyeing is continued at that temperature for a period of 45 minutes with frequent turning of the piece goods. The wool-modified cellulose acetate piece goods is then removed from the dye bath, and after rinsing and drying, yields a piece fabric which is dyed a uniform level solid red color.

**EXAMPLE VII.—(Wool-chrome dye)**

Cellulose acetate staple, containing 5% of polymerized beta-diethylaminoethyl alpha-methacrylate, is mixed with wool and converted by

standard procedures into a fabric containing 50% modified cellulose acetate and 50% wool. The mixed fabric after an aqueous scouring treatment is entered cold in a dye bath having a ratio of liquor volume to weight of fabric of 40:1 and containing 1% of a chrome dye (Anthracene Chromate Brown EB—Prototype No. 12), 15% of Glauber's salt and .1% of acetic acid. After turning the fabric frequently in the cold bath for 5 minutes, the temperature of the dye bath is raised to 85-90° C. in the space of 15 minutes and is held at that temperature for 45 minutes while the fabric is frequently turned. At the end of the 45 minutes, the fabric is lifted and 1% of chromic acid and 2% of acetic acid, dissolved in a small amount of cold water, are added to the dye bath. Once more the fabric is submerged in the dye bath and the temperature of the bath is raised slowly to 85-90° C. and maintained there for 30 minutes while the fabric is frequently turned. The wool-modified cellulose acetate fabric is withdrawn, rinsed, and dried. The finished fabric piece is dyed a uniform level brown color.

**EXAMPLE VIII.—(Silk-direct dye)**

A piece of velvet goods having a backing of natural silk and a pile facing of cellulose acetate yarns containing 10% of polymerized beta-diethylaminoethyl alpha-methacrylate is first submitted to the usual scouring treatment and then is entered at 50° C. into a dye bath having a ratio of liquor volume to fabric weight of 40:1 and containing 2% of a blue direct cotton dyestuff of Color Index No. 512, and 20% of Glauber's salt. The temperature of the dye bath is raised to 85° C. in the space of 15 minutes after which 5% of acetic acid is added. After 15 minutes at 85° C. and frequent turning of the velvet fabric, an additional 5% of acetic acid is added to the nearly exhausted dye bath and the dyeing continued for another 15 minutes. After removal from the dye bath, rinsing, and drying, the velvet exhibits a very satisfactory blue union between the silk backing and the modified cellulose acetate pile facing.

**EXAMPLE IX.—(Silk-acid dye)**

A piece of velvet goods having a pile facing of cellulose acetate containing 10% polymerized beta-diethylaminoethyl alpha-methacrylate and a backing of natural silk, is subjected to the customary scouring treatment and is entered at room temperature into a dye bath having a 40:1 ratio of liquor volume to fabric weight and containing 2% of a blue acid wool dye of Color Index No. 1088, 10% Glauber's salt, and 3% sulfuric acid. After 5 minutes at room temperature the dye bath is brought to 85° C. in the space of 15 minutes and dyeing continued at that temperature for 30 minutes while frequently turning the velvet goods. The velvet goods is then lifted, 1% of sulfuric acid is added, and the dyeing completed during the space of about 15 minutes while turning frequently the velvet fabric. After withdrawal, rinsing, and drying, a velvet fabric is secured showing a pleasing blue union between backing and pile facing.

**EXAMPLE X**

A mixed fabric consisting of a warp of cellulose acetate yarns containing 10% polymerized beta-diethylaminoethyl alpha-methacrylate, and a weft of regenerated cellulose threads, is dyed with a green vat dyestuff paste of Color Index No. 1101 in the following manner:

Twenty parts of the dye paste are mixed with 80 parts of the following composition:

5 550 parts of a boiled mixture comprising  
700 parts gum tragacanth (6%) and  
300 parts British gum powder  
190 parts potassium carbonate

Dissolve at 75° C., cool to 60° C. and add:

10 160 parts sodium formaldehyde sulfoxylate  
50 parts glycerin  
50 parts water.

The dye mixture is printed on the fabric, dried, aged for 4 to 6 minutes at 100° C. to 105° C. in an air-free ager, after which it is oxidized for 2 to 3 minutes at 45° C. to 55° C. in the following bath:

| Parts            |      |
|------------------|------|
| Sodium perborate | 5    |
| Water            | 1000 |

After oxidation, the printed mixed fabric is rinsed, soaped lightly, rinsed, and dried. If desired, the mixed fabric may first be dyed with a developed dye of a Color Index No. 317 and the fabric printed in the above fashion to secure a colored printed pattern on a differently colored background.

**EXAMPLE XI**

A mixed fabric, consisting of a warp of cellulose acetate yarns containing 10% of polymerized beta-diethylaminoethyl alpha-methacrylate, and a weft of regenerated cellulose yarns is dyed a blue color by the procedure of Example III with the blue developable dyestuff of Color Index No. 317. A white printed pattern on the blue background is produced with a printing paste prepared as follows:

| Parts                               |    |
|-------------------------------------|----|
| Zinc formaldehyde sulfoxylate conc. | 20 |
| Diethylene glycol                   | 15 |
| Water                               | 15 |
| Tragacanth gum (6% solution)        | 50 |

The paste is printed in the desired pattern on the dyed mixed fabric, dried, aged for 4 to 6 minutes at 100-105° C. in an air-free ager, rinsed, soaped, rinsed, and dried.

In all the above examples, unless otherwise specified, percentages are based on the weight of the mixed material being treated.

The process of the invention, consisting of modifying the cellulose acetate, producing a mixed material from the modified cellulose acetate and another fibre, and union dyeing the mixed material with a dyestuff having normally an affinity for the other thread but none for the cellulose acetate, is applied particularly advantageously to the production of solid colored effect on cellulose acetate mixed textile materials. However, it will be appreciated by the skilled technician that the process of the invention may also be applied with suitable variations broadly to union dyeing of mixed textile materials whenever it is desired that the cellulose acetate be definitely colored by the dyestuff selected for dyeing the other component fibre and having normally no affinity for cellulose acetate. Thus, by suitable variations of such factors as the temperature of the dye bath, the amount of modifier incorporated in the cellulose acetate, and the pH of the dye bath, the modified cellulose acetate fibre and the other component fibre or fibres of the mixed fabric may readily be colored to different depths to produce a pleasing colored cross dyeing effect 75 in a single dye bath, notwithstanding that the

dyestuff selected has no affinity for unmodified cellulose acetate.

While in the above examples, polymerized beta-diethylaminoethyl alpha-methacrylate has been used as the modifier, the process of the invention may be accomplished satisfactorily by the use of any other non-cellulosic, non-proteinous polymeric compound containing amino nitrogen, particularly an acetone soluble resinous one containing at least 2% amino nitrogen and soluble in 2% aqueous acetic acid but insoluble in water and 5% aqueous ammonia. Especially preferred as modifiers are the polymerized amino alcohol esters of acrylic acid containing a basic tertiary amino nitrogen group, such as beta-diethylaminoethyl alpha-methacrylate, beta-dimethylaminoethyl alpha-methacrylate, beta-piperidyl-N-ethyl-alpha-methacrylate, and beta-dicyclohexylaminoethyl alpha-methacrylate. As other suitable polymeric compounds containing amino nitrogen may be mentioned, non-cellulosic hexose amine polymer, such as deacetylated chitin; synthetic resins such as reaction products of phenol with aldehyde and ammonia or amines and resinous condensation polymers of amino dihydric alcohols with dibasic acids such as diethanol-methyleamine succinate and diethanolmethyleamine phthalate. As examples of the phenol-aldehyde-amine type resin may further be mentioned the reaction products between phenol, formaldehyde, ammonia, and dimethylamine; between phenol, lignin, formaldehyde, and dimethylamine; between phenol, formaldehyde, and dimethylaminoethanol; between phenol, formaldehyde, and dimethylol cyclohexanolamine; between phenol, formaldehyde, ammonia, and aniline; and many others.

Instead of simple polymers, interpolymers may be used, for instance, a reaction product of methylmethacrylate with methyl vinyl ketone in the presence of ammonium hydroxide or the reaction product of beta-cyclohexylaminoethyl methacrylate monomer with beta-dimethylaminoethyl methacrylate monomer under suitable conditions.

Preferably the modifier is incorporated in the spinning solution but it may also be incorporated in any other suitable manner in the cellulose acetate materials; for instance, the polymeric modifier may be dispersed in a suitable solvent or dispersing medium, the cellulose acetate material impregnated with the solution or dispersion, and the solvent or dispersing medium removed. In some cases, it may be desirable to incorporate the resin-forming components or monomer in the cellulose acetate structure and to form the resin in situ.

If the polymer is to be added to the spinning solutions, concentrations as high as 30% or even more, based on the weight of cellulose acetate, may be used. In general, however, concentrations ranging from about 3% up to about 15% or more are sufficient for most purposes. While it is possible to increase the depth of dyeing by larger quantities of the polymeric modifier, the increased dyeing depth is offset by weakening of the cellulose acetate structure.

The invention may be employed to secure colored effects throughout a mixed material, containing modified cellulose acetate, with most any dyestuff having little, if any, affinity for unmodified cellulose acetate; the only requisite is that the selected dyestuff have a natural affinity for the other thread component of the mixed material. Of the many classes and individual dye-

stuffs which have proven suitable may be mentioned as typical:

*Direct dyes*

5 Pontamine Scarlet B..... Color Index 382  
Pontamine Blue RWG..... Color Index 512

Also the direct dyes having the Color Index numbers 326, 533, 594, 415, 278, and 581.

10

Milling Red R..... Color Index 430  
Anthraquinone Blue Sky..... Color Index 1088  
Also acid dyes having Color Index numbers 15 667, 307, and 31.

*Developed color dyes (diazo dyes)*

Pontamine Diazo Black RS.... Color Index 552  
Pontamine Diazo Blue NA..... Color Index 317

20 Also developed dyes having Color Index numbers 401, 324a, and 1934 Yearbook Prototype 62.

*Chrome dyes*

25 Pontacyl Rubine R... Color Index 179  
Chromate Brown EB.. 1934 Yearbook Prototype 12

Also chrome dyes having Color Index numbers 216, 40, and 299.

30 All Color Index numbers appearing in the present specification are those given in the 1934 Yearbook of the American Association of Textile Chemists and Colorists.

It will be understood the dyeing conditions given in the above examples may be varied somewhat provided other factors are correspondingly adjusted. Likewise, in many cases, the dyeing conditions will have to be adjusted according to the characteristics of the particular dyestuff selected, the type of color effect desired, and the particular threads combined with the modified cellulose acetate in the mixed material. However, it is believed all such adjustments may be readily performed by following the principles outlined in the present invention. Generally speaking, the adjustments may be accomplished by suitable variation of all or part of the following factors: the amount of polymeric modifier incorporated in the cellulose acetate, the concentration of the dyestuff in the dye bath, the temperature of the dye bath, and the acidity or pH of the dye bath. Thus, for example, if a solid colored union is desired, and the modified cellulose acetate is being dyed too lightly, the condition may frequently be corrected by increasing the amount of polymeric amino containing modifier in the cellulose acetate. Again in certain cases such as where the other component of the mixed fabric is wool or silk, the differences may be eradicated by dyeing initially at an elevated temperature for a suitable period and then finishing the dyeing at a lower temperature, or vice versa dyeing initially at a lower temperature and finishing at an elevated temperature.

65 Most of the necessary dyeing control, however, is preferably attained through regulation of the acidity or pH of the dye bath. As pointed out in the above examples, such regulation may either be accomplished by changing the acidity by positive addition of suitable acidic or basic reagents during the union dyeing operation or by the use of a properly buffered dye bath. Generally speaking, it is essential in making the union dyed materials of the invention that at some stage in the dyeing the dye bath be somewhat acidic, for instance, of a pH between 6.9 and 5 and prefer-

ably between 6 and 5. In the case where the acidity is controlled by buffering the dye bath, most any of the buffering combinations or acid salts of phosphoric, boric, sulfuric, citric, carbonic, tartaric, or the like may be used to advantage. In cases wherein a progressive increase in acidity of the dye bath is desired, it is preferred to employ ammonium salts such as ammonium acetate or ammonium sulfate. Customary wetting agents used in dyeing operations may be present in the dye bath if desired.

It will be understood that the process of the invention may be applied advantageously to the dyeing in one bath of a mixed fabric of cellulose acetate and another material with a dyestuff having normally affinity only for the second material regardless of the physical form of the mixed materials. Thus, the modified cellulose acetate and the second material may be in the form of staple, fibres, threads, yarns, straws, ribbons, skeins, rovings, slivers, or woven and knitted fabrics such as suitings, crepes, velvets, hosiery, and car upholstery. Likewise, the modified cellulose acetate may be mixed with only one or with two or more materials depending as to whether a solid colored union is desired and in such case whether the materials added to the modified cellulose acetate can be dyed to substantially the same shade and color. With certain dyestuffs, the shade or color tone of the dye on the modified cellulose acetate component is somewhat different from that on the other component or components of the mixed material. Such is sufficiently satisfactory in many cases; if, however, a solid colored union of exactly matched shade and color tone is desired, it is possible to accomplish the same by addition of a proper auxiliary dyestuff having a natural affinity for the other component or components of the mixed material but none for unmodified cellulose acetate.

In discharge printing, where it is desired to secure a white pattern effect on a colored background, as well as in cases where the color is to be stripped substantially completely from the union dyed fabric, the zinc formaldehyde sulfonate, sodium formaldehyde sulfoxylate, or other discharge agent may be applied successfully either in the presence or absence of a swelling agent, such as zinc thiocyanate.

For convenience, the invention has been dis-

cussed in terms of cellulose acetate. The invention, however, is applicable also to other organic esters of cellulose, for instance, cellulose aceto-propionate, cellulose acetostearate, and cellulose propionate as well as cellulose ethers, such as methyl, ethyl, glycol, or benzyl cellulose in the same manner as above described with reference to the cellulose acetate.

Obviously, the cellulose acetate to be modified 10 and the mixed fabric dyed by the process of the invention may, if desired, contain besides the dye modifier, titanium dioxide or other inorganic and organic pigments as well as plasticizers, waxes, and similar substances.

15 Prior to the present invention, green and black solid unions were especially difficult to obtain. In contrast the process of the instant invention offers a relatively simple and inexpensive procedure of union dyeing cellulose acetate containing fabrics in essentially one dye bath by means of a dyestuff which has no affinity for unmodified cellulose acetate. By such means new 20 beautiful solid colored unions in cellulose acetate mixed materials may be secured over a wide range of colors and shades including greens and 25 blacks and in the most delicate and brilliant hues. A subsidiary advantage of the invention is the substantially complete exhaustion of the dyestuffs from the dye bath.

30 Many changes and modifications of the specific details hereinabove described can be made without departing from the nature and spirit of the invention, and it is, therefore, to be understood that the invention is not to be limited except as 35 set forth in the appended claim.

I claim:

The process of dyeing a mixed textile structure composed of cellulose acetate and a material other than cellulose acetate with a dyestuff 40 having an affinity for said other material but having substantially no affinity for said cellulose acetate material which comprises modifying said cellulose acetate material by the incorporation therein of a polymerized beta-diethylaminoethyl alpha-methacrylate whereby to impart thereto an 45 affinity for said dyestuff, forming said mixed textile structure with said modified cellulose acetate material, and dyeing said structure with said dyestuff.

WINFIELD WALTER HECKERT.

CERTIFICATE OF CORRECTION.

Patent No. 2,237,829.

April 8, 1941.

WINFIELD WALTER HECKERT.

It is hereby certified that error appears in the printed specification of the above numbered patent requiring correction as follows: Page 2, first column, line 33, for "after the" read --after which the--; page 4, first column, line 14, for "arcrylic" read --acrylic--; and that the said Letters Patent should be read with this correction therein that the same may conform to the record of the case in the Patent Office.

Signed and sealed this 13th day of May, A. D. 1941.

(Seal)

Henry Van Arsdale,  
Acting Commissioner of Patents.